

May 15, 1934.

A. H. STEWART

1,958,595

METHOD OF DECORATING ARTICLES

Filed June 27, 1932



Fig. 1.



Fig. 2.

INVENTOR

Andrew H. Stewart,  
By Archworth Martin,  
Attorney.

## UNITED STATES PATENT OFFICE

1,958,595

## METHOD OF DECORATING ARTICLES

Andrew H. Stewart, Shields, Pa., assignor to  
The Phoenix Glass Company, Monaca, Pa., a  
corporation of West Virginia

Application June 27, 1932, Serial No. 619,376

2 Claims. (Cl. 41—33)

My invention relates to a method of decorating articles, including sign globes for out of doors, such as those of the canteen type, and other surfaces—especially those intended for outside use.

It is common practice to decorate and letter the faces of sign globes by the decalcomania process, or by painting and then firing the colors. Because the decoration or lettering soon becomes 10 weather-worn and scales off, attempts have been made to preserve the applied color, by various means such as protecting plates of transparent glass, held against the decorated globe faces by cement and by metal fastenings, but these additional plates are expensive in the first instance 15 and also are fragile, so that replacements thereof are frequently necessary.

My invention has for one of its objects the provision of a new means and a method whereby 20 the decoration and lettering may be quickly and cheaply applied, and a transparent protective covering therefor employed that may be more conveniently applied than glass face plates.

Another object is to provide a transparent protective covering that is unbreakable and that will 25 cover the globe faces so snugly that dust is excluded therefrom, and which will not crack and peel off.

One of the forms which my invention may take 30 is shown in the accompanying drawing wherein Figure 1 shows a face view of a decorated globe, and Fig. 2 is a sectional view of one face thereof, taken on the line II—II of Fig. 1.

For convenience of description, I show a globe 35 3 of the canteen type which has flat or nearly flat faces 4 to which a transparent sheet of flexible material may be easily applied, without wrinkles, but surfaces other than flat surfaces can be protected by my method in the same manner, 40 and also sheets can be pre-formed to follow the contours of the surfaces.

The globe faces may be lettered and decorated 45 with colors in any suitable manner, but I prefer to employ the usual decalcomania or transfer process.

The decalcomanias are commonly transferred 50 from a paper sheet to which they are secured by water-soluble glue, to the surface to be decorated, by wetting the sheet. Glue adheres to the exposed side of the decalcomania, after transfer, and will assist in causing proper adhesion of the transparent facing sheets. After application of the decalcomania 5, and while it is still wet, I apply a sheet 6 of transparent water-proof "cellophane", a "kodapak", transparent water-proof

cellulose material, or the like, and press it firmly against the exposed decalcomania, by a roller or squeegee. The water is thereby squeezed from between the sheet and decalcomania and the sheet of course caused to fit snugly in place.

The facing sheets may, of course, be tinted in desired colors instead of being fully transparent.

If the decalcomania is permitted to dry before applying the transparent sheets, any suitable glue may be employed to attach the sheets thereto, or the decalcomania surface may be merely moistened with water and the transparent sheet applied to the moistened surface.

Instead of covering the decalcomania with transparent material that is initially of sheet form, I may paint it with a liquid material that will become a flexible sheet or film, when it dries. Various collodions are suitable for this purpose.

After the transparent sheet or film has been placed on the decorated surface, the article is 45 permitted to dry, and is then ready for use. However, it is preferable to subject the article, for several minutes, to a temperature of from 125° F. to 300° F., especially in those cases where sheets are employed. It has been found that this heating causes the protective covering to unite quite firmly with the decalcomania, without blistering, and that it will not peel off of the paint.

The upper limit of temperature will be under 50 that at which the facing will harden and crack or be melted, and under that at which the decalcomania material will melt greatly or be damaged.

In the case of the decalcomanias which I have 55 employed, globes containing the same have been heated to approximately 300° F., without causing excessive melting of the material. The softening of the decalcomania material, under heat, causes the transparent facing to adhere firmly thereto, independently of any residue of glue that may have been left on the exposed face of the decalcomania when the paper was removed.

The transparent facing sheets are superior to protective coatings of varnish or the like, because varnish not only cracks and peels with age, 60 especially by reason of heat created within interiorly-illuminated globes and by sun-rays, but the globes acquire a discolored appearance.

Instead of applying the decalcomania to the 65 glass surface and then placing the transparent sheet over the same, the decalcomania may initially be carried by the transparent sheet and applied to the glass surface by wetting the decalcomania or the glass, and pressing the transparent sheet and the decalcomania against the 70

glass. The globe may then be heated as heretofore explained, and this heating will not only effect a firmer union of the transparent sheet with the decalcomania material, but will also cause the decalcomania to adhere more firmly to the glass.

It will, of course, be understood that it is not essential for the transparent sheet to adhere to the face of the globe throughout the entire surface of the sheet, but the sheet can be pressed snugly against the globe and the edges thereof cemented or otherwise secured to the globe.

I claim as my invention:—

1. The method which comprises applying a de-

15

calcomania to a surface to be decorated, by wetting a sheet to which the decalcomania is attached by a water-soluble glue, removing the sheet and applying a transparent protecting sheet to the exposed surface of the decalcomania while the latter is still wet.

2. The method which comprises applying a decalcomania to a surface, applying a flexible transparent sheet to the decalcomania while it is wet, and sealing the edges of said sheet to the said surface.

ANDREW H. STEWART.

80

85

90

95

20

100

25

105

30

110

35

115

40

120

45

125

50

130

55

135

60

140

65

145

70

150

75